

Dec. 11, 1945.

J. A. MERRYMAN ET AL

2,390,805

METHOD OF MAKING METALLIC ARTICLES

Filed March 10, 1943

Fig. 1.



Fig. 2.



Fig. 3.



Fig. 4.



Fig. 6.



Fig. 7.



WITNESSES:

*Dick. C. Miller*

INVENTORS  
James A. Merryman &  
Edward M. Wharff, Jr.

BY

*James N. Ely*  
ATTORNEY

## UNITED STATES PATENT OFFICE

2,390,805

## METHOD OF MAKING METALLIC ARTICLES

James A. Merryman and Edward M. Wharf, Jr.,  
Wilkinsburg, Pa., assignors to Westinghouse  
Electric Corporation, East Pittsburgh, Pa., a  
corporation of Pennsylvania

Application March 10, 1943, Serial No. 478,642

2 Claims. (Cl. 117—65)

This invention relates to the method of producing metallic articles.

It is an object of this invention to provide a method of producing strong articles of spray metal.

Another object of this invention is to increase the strength of articles of spray metal without increasing the size of the article.

Other objects of this invention will become apparent from the following description when taken in conjunction with the accompanying drawing, in which:

Figure 1 is a view in elevation of a shaft having a worn end.

Fig. 2 is a view in elevation and partly in section of the shaft of Fig. 1 having spray metal applied thereto in accordance with the teachings of this invention.

Fig. 3 is an end view in section of the shaft of Fig. 2 with the layers of spray metal carried thereon.

Fig. 4 is an end view in section of the shaft carrying the spray metal after it has been subjected to a heat treatment in accordance with the teachings of this invention.

Fig. 5 is a view in section of apparatus illustrating the application of the teachings of this invention for the making of articles utilizing a removable form.

Fig. 6 is a photomicrograph at a magnification of 250 times of spray metal steel, and

Fig. 7 is a photomicrograph at a magnification of 250 times of the spray metal of Fig. 6 after having been treated in accordance with the teachings of this invention.

In accordance with this invention, metallic articles are produced by practicing the method of constructing the articles and heat treating them as explained more fully hereinafter. In industry, many metallic articles such as shafts or the like have worn surfaces which render such articles unsatisfactory for further service. Likewise, many castings have pits or flaws therein which render the casting unsatisfactory but which, if filled with a strong bonding metal, can be used commercially.

Referring to Fig. 1 of the drawing, there is illustrated a shaft 10 having a worn end or surface 12. In accordance with this invention, the worn surface 12 is roughened as by knurling or otherwise abrading it after which metal similar to the metal of the shaft 10 is sprayed thereon to deposit a layer 14 of spray metal of predetermined thickness as illustrated in Figs. 2 and 3. The method of spraying metal is well known in the art and need not be described herein, it being an established fact that the small particles of spray metal are mechanically bonded together by such methods.

In spraying the metal on the prepared surface 12, the spray metal mechanically links or interlocks with the roughened surface and is retained thereon. The spray metal deposit 14 can be readily controlled as to thickness, shape and size, the resulting structure being porous and having an oxide coating formed on the interlocking portions of the spray metal. When tested, such a deposit of spray metal is found to have only about half of the tensile strength of the solid metal before it is sprayed.

After the layer 14 of spray metal is deposited, the article carrying the spray metal is preferably heat treated in a reducing atmosphere of hydrogen or a mixture of hydrogen and nitrogen or other suitable reducing atmosphere to effect the reduction of the oxides formed during the spraying of the deposit 14. The length of time of heat treating the deposit in the reducing atmosphere to remove the oxides therefrom will vary depending upon the amount of oxides which are present.

When thus heat treated, a suitable brazing metal such as copper, or the well known copper base brazing alloys, or the like, are applied to the oxide-free deposit of spray metal. A preferred method of applying the brazing metal is to spray a layer 16 of the brazing metal over the external surface of the treated layer 14. The amount of brazing metal thus applied depends upon the thickness of the layer 14 as will be more apparent from the description given hereinafter.

After the layer 16 of brazing metal is applied to the layer 14, the shaft 10 carrying the spray metal is admitted to a brazing furnace (not shown) and is heated to a temperature above the melting point of the brazing material but below the melting point of the sprayed metal 14 and the shaft 10 in a reducing atmosphere, and maintained at such temperature for a sufficient length of time to permit the brazing material to completely impregnate the layer 14 and bond to the surface 12 of the shaft 10 as illustrated in Fig. 4. Upon examination it is found that the impregnated layer 14 is the same as it was prior to applying the layer 16. In other words, the brazing metal does not increase or otherwise change the size of the layer 14 when it fills the pores thereof.

By effecting the impregnation in a reducing atmosphere, all oxides present in the layers of spray metal are effectively reduced and complete impregnation is obtained if the layer 16 of brazing metal is of a thickness sufficient for supplying enough of the brazing metal for such impregnation. Of course, an excess of brazing metal is a waste remaining on the surface of the layer 14 or flowing therefrom in the furnace. Any excess of the brazing metal remaining on the surface of the layer 14 can be readily machined

therefrom. By tests, the optimum and minimum thickness of the layer 14 can be determined for different thicknesses of the layer 14 for obtaining the complete impregnation of the layer 14 and the bonding to the surface 12 of the shaft 10.

In another embodiment of this invention, the layer 14 of spray metal is applied to a removable form 18 as illustrated in Fig. 5 of the drawing. In this embodiment the form 18 is of graphite or other suitable refractory material, and is designed to have the predetermined shape and size of the article which is to be produced. The layer 14 is readily sprayed onto the form 18 to any predetermined thickness and is thereafter treated in a reducing atmosphere to effect the reduction of any oxides. In this embodiment the brazing metal may be applied to the layer 14 as by spraying as described with respect to the embodiment shown in Figs. 1 through 4, or the brazing metal in the form of the pellets 20 or the like may be positioned on the layer 14 as illustrated in Fig. 5. The pellets 20 may thus be positioned while the coated form is in the reducing atmosphere, the temperature of the furnace then being increased to a temperature above the melting point of the brazing metal and maintained at such temperature to insure the complete impregnation of the porous metal layer 14. Preferably the article is then cooled in the reducing atmosphere to below 200° C. to prevent the formation of oxides. When thus formed, the impregnated layer 14 is readily stripped from the form 18 to give a strong article of required shape and size.

In actual practice, it may be preferred to apply a thicker layer 14 of the spray metal than is actually required, and after impregnating the layer 14 with the brazing metal to machine the impregnated layer to the exact size of the required article. This can readily be accomplished as the impregnated layer can be as readily machined as the base metal.

Referring to Figs. 6 and 7 of the drawing, there is illustrated photomicrographs of sprayed steel of the type of the layer 14 and of the same steel after having been impregnated with copper.

Fig. 6 in particular is a photomicrograph at a magnification of 250 times of sprayed SAE steel #1010, and clearly illustrates the effect of spraying the steel in that impurities are included and the steel is deposited substantially in layers. Such sprayed steel, when subjected to the Izod impact test, had a strength of only one foot-pound as sprayed.

When treated as described hereinbefore and impregnated with copper, the steel has an entirely different characteristic as illustrated in Fig. 7. This figure is a photomicrograph of the impregnated sprayed steel at a magnification of 250 times. As illustrated, there are very little impurities entrapped in the steel and the copper utilized as the brazing material completely impregnates the porous structure of the sprayed steel. The impregnated sprayed steel illustrated in Fig. 7 has an Izod impact strength of 50 foot-pounds. Such improvement in the strength of the impregnated sprayed steel over the steel as sprayed is remarkable and clearly illustrates the value of the present invention, similar results being obtained in other sprayed articles. Even

where the sprayed steel is not completely impregnated, a remarkable improvement in strength is obtained, for, in another article in which insufficient copper was employed for impregnating the sprayed metal, the strength of the brazed-spray metal increased from one foot-pound to 15 foot-pounds when impregnated even though the article had a porous structure.

In general, the impregnation of the sprayed metal layer can be efficiently effected by subjecting the sprayed metal to a temperature of between 1900 and 2100° F. in a reducing atmosphere for a period of time of from 1 to 2 hours to insure the removal of oxides, and, after the copper or other brazing material is applied to the oxide-free sprayed metal, subjecting the article to a temperature of between 2000 and 2300° F. in the reducing atmosphere for a period of time of from 10 minutes to 1½ hours, depending upon the size of the article.

This invention is particularly applicable to the reclaiming of shafts, tools or the like which have been damaged in service, or to castings which have pits and flaws or chips therein. The portions of the article which have been rebuilt by applying the spray metal and treated in accordance with this invention have unusual strength and makes it possible to utilize the articles in industry where otherwise they would be normally discarded.

Although this invention has been described with reference to a particular embodiment thereof, it is, of course, not to be limited thereto except in so far as is necessitated by the scope of the appended claims.

We claim as our invention:

1. The method of making metallic articles comprising, in combination, spraying low carbon steel to deposit and form a spray metal article having a porous structure, heating the sprayed steel to a temperature of between 1900° F. and 2100° F. in a reducing atmosphere for a period of time ranging from one to two hours to reduce any oxides present thereon, applying a brazing metal selected from the group consisting of copper and copper base alloys to the heat treated article, and subjecting the article to a temperature of between 2000° F. and 2300° F. in a reducing atmosphere for a period of time sufficient to permit the brazing metal to penetrate and substantially fill the pores of the sprayed steel.

2. The method of making metallic articles comprising, in combination, spraying low carbon steel to deposit and form a spray metal article having a porous structure, heating the sprayed steel to a temperature of between 1900° F. and 2100° F. in a reducing atmosphere for a period of time ranging from one to two hours to reduce any oxides present thereon, spraying a brazing metal selected from the group consisting of copper and copper base alloys onto the heat treated sprayed steel, and subjecting the sprayed composite metal to a temperature of between 2000° F. and 2300° F. in a reducing atmosphere for a period of time ranging from ten minutes to one and one-half hours to permit the brazing metal to penetrate and substantially fill the pores of the sprayed steel.

JAMES A. MERRYMAN.  
EDWARD M. WHARFF, JR.